

## UNITED STATES PATENT OFFICE

2,017,488

## ARC WELDING ELECTRODE

Lionel E. Faulkner, Hillside, N. J., assignor to  
 Wilson Welder & Metals Company, Inc.,  
 Hoboken, N. J., a corporation of New York

No Drawing. Application March 3, 1934,  
 Serial No. 713,881

8 Claims. (Cl. 219—8)

This invention relates to electrodes for metallic-arc welding, and more particularly to that type of welding electrodes, having a relatively thick coating, which are used in the so-called 5 "shielded-arc" process.

Coated electrodes are usually in the form of a short length of metal rod or wire to which the coating has been applied by any suitable process, such as by extrusion through a die or by dipping. In use, the arc is struck between the metal rod and the work, the rod melting in the heat of the arc and being deposited on the work. The coating usually contains suitable fluxing, deoxidizing and slag-forming materials, together with 10 a binder to make them adhere together and to the rod, for reasons well understood in the art. The advantages of this type of electrode may briefly be stated to be: (1) an increased rate of deposit by permitting the use of a higher current, (2) avoidance of a so-called "wild arc", 15 (3) decrease of spattering, (4) better penetration of the work by the deposited metal, (5) greater density and homogeneity of deposited metal with avoidance of pinholes, and (6) generally improved quality and strength of the 20 weld.

Such coatings are either melted or consumed by the intense heat of the arc, depending upon 25 their ingredients, some of which may be combustible. The weld is improved because the coating is so constituted as to form a shield around the end of the rod as it melts so that the arc is projected from a crucible resulting 30 from the consumption of the rod more rapidly than the coating, the coating which projects beyond the end of the rod helping to protect the molten metal from contact with the air. As 35 the coating is melted and consumed, the non-combustible constituents cover the surface of the deposited metal with slag. This slag cover 40 protects the metal while molten from the harmful effects of the air, to which it is susceptible while in the fluid state, and prevents the formation of scale after the metal solidifies and before 45 it has cooled. It also slows the cooling of the deposited metal.

Many heavily coated electrodes present the 50 difficulty of leaving a deposit of too much slag, which runs into the arc, particularly when the weld is being made in positions other than horizontal. This may cause the arc to go out and 55 may cause a fault in the weld. Moreover when the arc is extinguished the slag may seal over the end of the electrode, forming an insulation

which must be broken off before the arc can be started again.

By this invention new and improved electrode coatings are provided which furnish the correct amount of shield without an excess of slag. 5 The coatings hereinafter described are characterized by the fact that they contain, among their ingredients, pyrogenous residues, particularly pitches and asphaltites, the latter being native pyrogenous substances. As to pitches, 10 excellent results have been obtained using pitches derived from the destructive distillation of wood, fatty-acid pitches, and coal-tar pitches. As an example of an asphaltite, gilsonite has given good results. Hardwood-tar pitch has 15 been found especially well suited for the purpose. An example of a formula for a coating, using hardwood-tar pitch, is as follows:

| Ingredient—              | Parts by weight |
|--------------------------|-----------------|
| China clay               | 20              |
| Powdered asbestos        | 20              |
| White sercrite mica      | 35              |
| Pumice                   | 10              |
| Hardwood-tar pitch       | 10              |
| Silico manganese         | 25              |
| Iron oxide ( $Fe_3O_4$ ) | 18              |
|                          | 20              |

to which is added about 43 parts by weight of sodium silicate ( $Na_2O : SiO_2$  ratio 1 to 3.22) of 30 about 40-42° Baumé to make the mixture into the consistency of dough for extruding. The dry materials are finely ground before mixing. The coating as above prepared is extruded through a die onto a bare wire of about .156 35 inch diameter, the coated rod being about .190 inch diameter. A rod of .187 inch diameter would be coated to .240 inch diameter. These coating sizes may be varied, however, to make the rods suitable for various types of work. 40

An example of a formula for a coating using gilsonite, an asphaltite, is:

| Ingredient                                      | Parts by weight |
|-------------------------------------------------|-----------------|
| Zinc oxide                                      | 20              |
| Ilmenite                                        | 45              |
| Iron oxide ( $Fe_3O_4$ )                        | 20              |
| Pumice                                          | 20              |
| Gilsonite                                       | 10              |
| Asbestine                                       | 10              |
| Silico manganese                                | 5               |
| Magnesium oxide                                 | 50              |
| White sercrite mica                             | 18              |
| Calcium carbonate                               | 1               |
|                                                 | 35              |
| To the above are added about 80 parts by weight | 20              |
|                                                 | 55              |

of sodium silicate of about 40-42° Baumé to make a dough applied to the metal rod as stated above.

In the second formula various types of pitch may be substituted for the gilsonite, using the same weight of substituted material. Fatty-acid pitches such as vegetable stearine pitch and bone pitch, hardwood-tar pitch and coal-tar pitch produce similarly satisfactory results. These pitches are preferably such pyrogenous residues as come from distillation which produces a pitch which is brittle at room temperatures and readily pulverized to the desired fineness for mixing with the other ingredients. The hardwood-tar pitch used, for example, has a flow point of about 15 85° C., but the flow point is not significant except as it is such as to permit the pitch to be pulverized.

While these formulae are given as examples of coatings which produce highly satisfactory results, the invention is not limited to the ingredients or proportions specified. The quantity of pitch or asphaltite in particular may be varied in order to increase or decrease the relative amount of the coating which is consumed by the heat of the arc and to correspondingly decrease or increase the relative amount of slag-forming material in the coating, while retaining the desired shield for the arc. To maintain the proper thickness of shield without an excessive deposit of slag is very desirable, particularly when welding in positions other than flat, that is, in vertical or overhead welding. This invention contemplates that the amount of pitch or asphaltite may be varied from the amounts given in the above formulae within wide limits. For example, in the first formula set forth above the amount of hardwood tar pitch may readily be doubled, with only slight adjustment of the quantities of the other ingredients in the coating to maintain the proper consistency of coating material and of the slag produced in the arc. It will be noted that by reason of the relatively low specific gravity of the pitch etc., doubling the weight of pitch given in the illustrative formulae will result in a relatively larger increase in the volume of combustible material in the coating.

Binders other than sodium silicate may be used, for example, potassium silicate, glue, dextrine paste or vegetable gum such as gum tragacanth or gum arabic. Another method of applying the coating is to mix the dry ingredients, including the pitch or asphaltite, and heat the mixture to the melting point of the pitch or asphaltite, applying it to the rod while in that condition and allowing it to cool.

The foregoing description is illustrative of several embodiments of the invention, which is not intended to be limited thereby.

What is claimed is:

60 1. An arc welding electrode comprising a metallic rod having a coating of fluxing, deoxidizing, and slag-forming materials, including a quantity of a pyrogenous residue of organic materials in-

corporated in said coating and proportioned in amount relative to the other ingredients so that the coating will produce in the heat of the arc the desired amount of slag while maintaining a shield for the arc.

2. An arc welding electrode comprising a metallic rod having a coating of fluxing, deoxidizing, and slag-forming materials, including a quantity of a pitch incorporated in said coating and proportioned in amount relative to the other ingredients so that the coating will produce in the heat of the arc the desired amount of slag while maintaining a shield for the arc. 10

3. An arc welding electrode comprising a metallic rod having a coating of fluxing, deoxidizing, and slag-forming materials, including a quantity of an asphaltite incorporated in said coating and proportioned in amount relative to the other ingredients so that the coating will produce in the heat of the arc the desired amount of slag while maintaining a shield for the arc. 15

4. An arc welding electrode comprising a metallic rod having a coating of fluxing, deoxidizing, and slag-forming materials, including a quantity of gilsonite incorporated in said coating and proportioned in amount relative to the other ingredients so that the coating will produce in the heat of the arc the desired amount of slag while maintaining a shield for the arc. 25

5. An arc welding electrode comprising a metallic rod having a coating of fluxing, deoxidizing, and slag-forming materials, including a quantity of coal-tar pitch incorporated in said coating and proportioned in amount relative to the other ingredients so that the coating will produce in the heat of the arc the desired amount of slag while maintaining a shield for the arc. 30

6. An arc welding electrode comprising a metallic rod having a coating of fluxing, deoxidizing, and slag-forming materials, including a quantity of a fatty-acid pitch incorporated in said coating and proportioned in amount relative to the other ingredients so that the coating will produce in the heat of the arc the desired amount of slag while maintaining a shield for the arc. 40

7. An arc welding electrode comprising a metallic rod having a coating of fluxing, deoxidizing, and slag-forming materials, including a quantity of a wood-tar pitch incorporated in said coating and proportioned in amount relative to the other ingredients so that the coating will produce in the heat of the arc the desired amount of slag while maintaining a shield for the arc. 45

8. An arc welding electrode comprising a metallic rod having a coating of fluxing, deoxidizing, and slag-forming materials, including a quantity of hardwood-tar pitch incorporated in said coating and proportioned in amount relative to the other ingredients so that the coating will produce in the heat of the arc the desired amount of slag while maintaining a shield for the arc. 50

LIONEL E. FAULKNER.